

Jan. 4, 1944.

H. PULFRICH ET AL

2,338,538

GLASS-TO-METAL SEALS

Filed June 1, 1939

Fig. 1.



Fig. 2



Inventors:  
Hans Pulfrich,  
Richard Magner,  
by Harry E. Shulam  
Their Attorney.

## UNITED STATES PATENT OFFICE

2,338,538

## GLASS-TO-METAL SEAL

Hans Pulfrich, Berlin-Friedenau, and Richard  
Magner, Berlin, Germany, assignors to General  
Electric Company, a corporation of New York

Application June 1, 1939, Serial No. 276,928  
In Germany July 11, 1938

6 Claims. (CL. 49—92)

The present invention relates to glass-to-metal seals and more particularly to an improved method and means for sealing glass to iron.

In joining iron to glass parts, considerable difficulty is experienced in securing satisfactory adherence of the iron and glass surfaces. We have found that this difficulty may be substantially lessened by coating the iron with a layer of cobalt or molybdenum (preferably cobalt) and then annealing until an alloy is formed. Our invention in this connection may best be understood by reference to the following description and the accompanying drawing in which Figs. 1 and 2 represent exemplary embodiments of the invention.

In order to produce an adherence-improving coating of cobalt or molybdenum on an iron body it is convenient to apply the coating material by electrolytic deposition so as to form a plating. The coated iron part is then annealed from one to five hours at 1000 to 1400 degrees C. this being preferably done in a neutral gas such as hydrogen.

The above specified heat treatment causes the cobalt (or molybdenum) to be diffused into the iron, resulting in the production of an inhomogeneous surface layer of alloy. Such layer is found to possess a cobalt content which diminishes in the direction of the normal line from the surface to the interior of the part. We prefer to continue the heating procedure until the alloyed layer contains from 15 to 30% of cobalt at its outer surface. Within this range the coefficient of expansion of the iron part is not seriously affected by the addition of the cobalt.

For sealing with a metal part prepared in accordance with our invention, one may employ a so-called soft glass, i. e., a glass with a coefficient of thermal expansion of from  $80 \times 10^{-7}$  to  $100 \times 10^{-7}$  centimeters per centimeter per degree centigrade. One example of such a glass comprises the so-called Sendlinger glass which is free from lead and which contains a substantial quantity of barium oxide. This glass has a coefficient of expansion of about  $95 \times 10^{-7}$ .

In Fig. 1 we have shown our invention as applied in connection with a seal which comprises a metal sleeve 1, a body of glass 2, and a lead-in wire 3 which passes through the body of glass. The sleeve is preferably constituted of iron having an alloyed surface prepared in accordance with the method described in the foregoing. The conductor 3 may be of similar composition if desired.

We have found that superior results are ob-

tained when the coefficient of expansion of the conductor 3 is from 1% to 10% above the coefficient of expansion of the glass. We consider it especially advantageous to use for the conductor an alloy of from 40 to 50% iron with from 60 to 50% nickel, such alloy being provided with a superficial addition of cobalt or molybdenum (specifically, 1 to 5%) to improve adhesion.

Referring again to Fig. 1, the density of the stippling applied to the sleeve 1 is an indication of the varying concentration of the coating metal from point to point in the iron. It will be noted that the sleeve is alloyed only on its inner side, the outer side being preferably free from coating in order to facilitate welding of the sleeve to other metal parts.

In Fig. 2 there is shown a sleeve provided with an annular flange 5. In this case the cobalt or molybdenum coating is preferably applied only to the cylindrical portion 6 of the sleeve, being excluded, for example, from the surface of the flange 5.

What we claim as new and desire to secure by Letters Patent of the United States is:

1. A glass-to-metal seal including a body which consists mainly of iron, the outer layer of said body comprising an alloy of iron with a metal selected from the group consisting of cobalt and molybdenum, and a body of glass adhering to said alloy layer.

2. A glass-to-metal seal including a body which consists mainly of iron, the outer layer of said body comprising an alloy consisting substantially of iron and cobalt, and a body of glass fused to said layer, the content of cobalt in the alloy layer at the region of fusion with the glass being from about 15% to about 30%.

3. A lead-in arrangement including a tubular iron sleeve having a layer of cobalt-iron alloy on the interior surface thereof, the cobalt content of said layer diminishing inwardly from the surface, a body of glass within the sleeve and sealed to the surface of said layer, and a conductor sealed through said glass and supported thereby in spaced relation to the sleeve, the content of cobalt in the said cobalt-iron layer at the region of fusion with the glass being from about 15% to about 30%.

4. A lead-in arrangement comprising a tubular iron sleeve having a layer of cobalt-iron alloy on the interior surface thereof, the cobalt content in said layer diminishing toward the interior of the sleeve wall, a body of glass within the said sleeve and sealed to the surface of the said layer, a conductor sealed through said glass

and supported thereby in spaced relation to the sleeve, and a laterally extending flange at one end of the said sleeve, the surfaces of said flange being free of cobalt to facilitate welding of the flange to other metallic parts.

5. A glass-to-metal seal including a metal body, the outer layer of said body comprising an alloy of iron and cobalt and a body of glass fused to the surface of said alloy layer, the content of cobalt in the alloy at the glass surface being about 15 10 to 30 per cent and the cobalt content diminishing from the surface toward the interior.

6. A body of glass having a coefficient of expansion of about  $80$  to  $100 \times 10^{-7}$  cm. per cm. per degree centigrade, a conductor sealed thereto which comprises an alloy of 40 to 50% iron and 60 to 50% nickel, and having the sealing surface thereof which is joined to said glass body alloyed with a metal chosen from the group comprising cobalt and molybdenum.

HANS PULFRICH.  
RICHARD MAGNER.